

June 22, 1943.

I. W. A. KIRKWOOD ET AL

2,322,215

ELECTRIC CONDENSER BUSHING

Original Filed June 13, 1939



Impregnating Polymerizable  
Liquid Substantially  
Polymerized



INVENTOR  
Sam W. A. Kirkwood  
Patrick D. Ritchie  
BY  
Hanson, Cole, Grindle & Hanson  
ATTORNEY

## UNITED STATES PATENT OFFICE

2,322,215

## ELECTRIC CONDENSER BUSHING

Ian Ward Anderson Kirkwood and Patrick Dunbar Ritchie, Newcastle-on-Tyne, England, assignors to A. Reyrolle & Company Limited, Hebburn-on-Tyne, England, a company of Great Britain

Original application June 13, 1939, Serial No. 278,965. Divided and this application April 23, 1942, Serial No. 440,222. In Great Britain June 14, 1938

12 Claims. (Cl. 174—143)

This application is a division from our application, Serial No. 278,965, filed June 13, 1939.

This invention relates to electric condenser bushings.

Electric insulating bushings which consist of superimposed layers of a cellulosic base, such for example as paper or cloth, with one or more stress-grading conducting foils between the layers which are bonded with synthetic resins or other binders are subject to the disadvantage that they are liable to absorb moisture, since cellulosic materials, in general, are inherently hygroscopic. Even if the cellulosic insulator is impregnated with a synthetic resin the absorption of moisture by the fibres will not be wholly prevented and there will ultimately be a decrease in the dielectric strength, increase of power factor, and swelling of the insulator at the exposed ends of the fibrous layers.

The main object of the present invention is to overcome this disadvantage by forming a condenser bushing of materials which are essentially non-hygroscopic.

A further object of the invention is to provide a condenser bushing comprising a plurality of concentric superimposed layers of fibres of a vitreous substance, at least one stress grading conducting foil between adjacent vitreous layers and a solid insulating medium filling the interstices in the vitreous layers, the insulating medium having a dielectric strength within the interstices exceeding that of air at atmospheric pressure.

It is desirable that the vitreous substance employed be uniform in structure and free from incorporated foreign matter, that it will provide individual fibres of a satisfactory textile length, and that it will be wholly (or substantially wholly) non-hygroscopic.

In order to facilitate filling of the interstices between the fibres with the insulating medium the fibres may be bound together in open texture by a preliminary binder prior to filling of the interstices with the insulating medium.

According to a further object of the invention the interstices in the fibrous layers are filled with an insulating binder, such for example as a phenol-formaldehyde resin, a higher chlorinated naphthalene, or shellac applied in solution or, in certain cases where this is possible, in liquid or semi-liquid state. The insulating binder may be applied to the fibres prior to the winding or wrapping which is then effected under the application of pressure and/or heat so that the layers are impregnated with the binder which binds the

layers into a solid mass. Alternatively, the fibres (preferably bound in open mesh by a preliminary binder as above described) are first wound or wrapped and the interstices are then filled with the insulating binder, as by dipping the wound or wrapped layers in the insulating binder while this is in a liquid or semi-liquid state.

According to yet a further object of the invention the interstices in the wound or wrapped layers are filled by impregnation, preferably in vacuo, with a polymerisable liquid, such for example as styrene, this liquid being then polymerised by heating, if necessary under pressure. Thus, for example, the liquid impregnant may be forced through the insulating mass from end to end so as to force out the air and fill the interstices with the impregnant.

With a view to imparting flexibility as may be desired a suitable plasticizer may, in any of the above methods, be incorporated in the insulating binder.

In the accompanying drawing

Figure 1 illustrates one method of forming a condenser bushing according to the invention,

Figure 2 shows the finished bushing in longitudinal section,

Figure 3 illustrates another method according to the invention, and

Figure 4 shows the finished bushing in longitudinal section.

In Figure 1 the bushing is formed by applying to a cord or a strip of felted glass wool or woven glass cloth, for example a glass wool fabric, a binder constituted by phenol formaldehyde resin, polystyrene or polyvinyl acetal. The strip or cord A thus treated or "varnished" is dried and then wrapped in a number of superimposed layers A<sup>1</sup> about a former B, which may be a conductor, with the insertion of stress-grading foils C between the layers A<sup>1</sup> as they are wound. The layers A<sup>1</sup> with the foils C between them are subjected to heat and pressure by rolls D so that the interstices in and between the layers A<sup>1</sup> are impregnated with the binder and the insulation is thus bound into a solid mass about the former or conductor B as shown in Figure 2.

In accordance with a second method, as shown in Figure 3, a cord or a strip of felted or woven glass wool A<sup>3</sup> is first wrapped round a conductor or former B<sup>1</sup> in a number of superimposed layers A<sup>4</sup>, stress-grading elements C<sup>1</sup> being inserted between the layers A<sup>4</sup> as they are wound. The layers are then impregnated, preferably in vacuo, with a polymerisable liquid such for example as styrene or methyl methacrylate, or solutions

therein of the corresponding polymers. The liquid is then polymerised by the application of heat, if necessary under pressure to avoid formation of bubbles. The finished bushing is shown in Figure 4.

According to a modified method the cord or strip of woven or felted glass wool A (Figure 1) wound in a number of superimposed layers about a conductor or former with stress-grading foils C between them, is dipped or otherwise impregnated, preferably in vacuo, with a molten wax-like material, such for example as chlorinated naphthalene or ceresine, which on cooling will set to bind the fibres into a solid mass.

According to another modification a cord or strip of glass cloth, for example felted or woven glass wool has applied thereto shellac, a natural wax, a chlorinated naphthalene or a phenolic, urea, vinyl or acrylic resin, each in a suitable solvent which is then removed in known manner. A cord or fibrous strip thus treated is wound or wrapped in a number of superimposed layers about a conductor or former as described with reference to Figure 1, metal foils being inserted between adjacent layers as they are wound and subjected to simultaneous heat and pressure by the rolls D.

In order to impart flexibility as may be desired a suitable plasticiser, such for example as chlorinated diphenyl, amyl naphthalene, dibutyl phthalate, or tricresyl phosphate, may in each of the above methods be incorporated in the binder.

Impregnation of the interstices between the fibres will be facilitated if the texture of the fibrous layers is as open as may be practicable. Though it is a matter of some difficulty to weave a fibre-glass textile of loose open mesh owing to warp-slip, this difficulty may be overcome by using, for example in any of the methods above described, a felted mat of glass fibres held together by a small quantity, say 1% to 2% by weight, of a preliminary binder such for example as phenol-formaldehyde resin or polystyrene, the binder content being just sufficient to hold the fibres against slip at their main points of mutual contact. This gives an open-textured material which will be readily permeated by the liquid impregnant. Alternatively a felted mat as described may be employed, for example with the first and fourth methods above described, in which the preliminary binder content is high, for example 40% to 60% by weight of the whole, so that, after winding or wrapping, impregnation of the felted mat by the binder can be effected by hot-pressing or hot-rolling the superimposed layers. If a thermoplastic binding is employed with this method careful control of the tension to which the material is subjected during winding or wrapping should be exercised in order to avoid undesirable stretching.

The felted mat, incorporating the binder, may be formed for example by agitating a suspension of short fibres of a vitreous substance (e. g., glass wool) in a reaction mixture giving rise to a synthetic resin. For example, the fibres may be stirred into a heated mixture of phenol and aqueous formaldehyde in suitable proportions. When the condensation has proceeded to the point where the reactants have formed an A-stage phenolic resin (resole) the whole is poured out on to a smooth, endless conveyor belt, forming a thin film from which all surplus water is carefully evaporated, if desired under reduced pressure. The resulting film may then be wound

into a bushing in the usual manner under the action of heat and pressure.

It will be understood that the electrical, mechanical, and other properties of the bushing produced in accordance with the invention may be modified to suit requirements and conditions of use, by suitable selection not only of the vitreous material but also the filler or binder. Thus, a lead glass will usually give a lower power factor and a higher dielectric constant than a soda-lime glass, but both possess a surface which is somewhat susceptible to atmospheric moisture. The thickness of the layer of moisture which can be adsorbed on the surface of the fibres will depend upon their chemical composition, such thickness usually decreasing, for example, with decrease of the soda and increase of the boric oxide content of the fibres. It is in general preferred to employ the substantially alkali-free boro-silicate glass fibres already available in the industry, but a particularly desirable combination of materials, from the dielectric standpoint, comprises vitreous silica fibres impregnated or bound with a hydrocarbon such as polystyrene, or a polymerised ethylene plastic. When employing woven fibres the warp may differ chemically or otherwise from the weft, so as to produce intentional differences, in two mutually perpendicular directions, of various characteristics, such for example as elasticity. When the lowest possible power-factor is required, it is desirable that the fibres be as free as possible from the emulsions of oil, starch, and other materials with which they are usually moistened during spinning into thread form. These materials usually contain emulsifying agents which, though present only in minute amount on the final weave, are polar compounds which could with advantage be removed, prior to the application of the binder or impregnant, for example by washing with water, trichlorethylene or other suitable solvents or vapours thereof, followed by intensive drying.

The vitreous substance employed in accordance with the invention has no inherent tendency to absorb moisture and, though it may tend to adsorb a surface layer of moisture from a humid atmosphere, this layer can readily be removed by heating prior to the fibres being "filled" or bound to form the bushing. For this purpose, by using an inorganic vitreous substance, a higher temperature can safely be employed than with cellulosic materials which will only withstand a comparatively low temperature. Further, whereas a cellulosic material, such as paper, coated with polystyrene, can be pressed into laminated sheets at temperatures of about 120° C. to 160° C., paper coated with polymerised N-vinyl carbazole would require a temperature of about 250° C. to 300° C. in order to render the binder sufficiently plastic to flow readily into the interstices. This would, however, damage the paper and render it brittle. By employing an inorganic vitreous substance instead of cellulosic material much higher manufacturing temperatures can safely be applied. Again, bushings composed of cellulosic materials bound with phenolic resins are readily "tracked," that is to say they produce a carbonised conducting track when brought into contact with an electric arc. This tendency can be reduced by substituting a urea for a phenolic resin, or glass for cellulosic material. It can be substantially eliminated in an insulating body according to the invention using glass fibres bound with a urea or

other non-tracking plastic since an arc will merely cause fusion of the surface fibres.

It will be understood that the application of the insulating filler or binder may be effected either before or after winding or wrapping of the successive layers of the vitreous substance. For example, the vitreous substance may be varnished with a thermo-setting varnish before winding on the conductor or former, or the layers may be wound before the interstices are filled, say by a monomer which is subsequently polymerised, or a syrupy solution of a polymer in a monomer may be applied to the vitreous substance before winding the layers on the conductor or former and then polymerising.

In any of the methods above described the filler or binder may be applied as an emulsion or suspension of globules or particles of the filling or binding medium in an immiscible liquid.

The superimposed layers may be formed from a textile fabric woven from spun fibres or threads of the vitreous substance. These layers may also be formed by winding thin fibres, sheets, irregular layers similar to felt, or extruded woven or braided cord, made of the said vitreous substance.

What we claim as our invention and desire to secure by Letters Patent is:

1. An electric condenser bushing comprising a plurality of concentric superimposed layers of fibres of a vitreous substance, at least one stress grading conducting foil between adjacent vitreous layers and a solid insulating medium filling the interstices in the vitreous layers, the insulating medium having a dielectric strength within the interstices exceeding that of air at atmospheric pressure.

2. An electric condenser bushing comprising a conductor, a strip of glass wool wound in a number of superimposed layers about the conductor, at least one stress-grading conducting foil between adjacent layers, and a resinous filler filling the interstices in the layers so as to bind the whole into a compact mass about the conductor.

3. An electric condenser bushing as claimed in claim 2 in which the resinous mass contains a plasticiser.

4. An electric condenser bushing comprising a

plurality of concentric superimposed layers of woven fibres of a vitreous substance, at least one stress grading conducting foil between adjacent vitreous layers and a polymerised binder filling the interstices in the layers, the binder having been polymerised in the assembled bushing so as to bind the whole into a compact mass about the conductor.

5. An electric condenser bushing comprising a conductor, a series of superimposed layers consisting of a strip of glass-wool fibres wound on the conductor, at least one stress-grading conducting foil between adjacent layers, and a phenol-formaldehyde resin filling the interstices in the strip and polymerised so as to bind the whole into a compact mass about the conductor.

6. An electric condenser bushing as claimed in claim 1, in which the insulating medium consists of a polymerised aromatic hydrocarbon of the vinyl type.

7. An electric condenser bushing as claimed in claim 1, in which the insulating medium consists of polyvinyl acetal.

8. An electric condenser bushing comprising a conductor, a series of superimposed layers of glass-wool fibres on the conductor, at least one stress-grading conducting foil between adjacent layers, and a polymerised electrically insulating binding material containing a plasticiser filling the interstices in the layers.

9. An electric condenser bushing as claimed in claim 8, in which the plasticiser consists of amyl naphthalene.

10. An electric condenser bushing as claimed in claim 8, in which the binding material consists of a polymerised aromatic hydrocarbon of the vinyl type with a plasticiser of amyl naphthalene.

11. An electric condenser bushing as claimed in claim 8, in which the plasticiser consists of chlorinated diphenyl.

12. An electric condenser bushing as claimed in claim 8, in which the binding material consists of a polyvinyl acetal with a plasticiser of chlorinated diphenyl.

IAN WARD ANDERSON KIRKWOOD.  
PATRICK DUNBAR RITCHIE.